

## UNITED STATES PATENT OFFICE.

BERTRAM T. MCBAIN, JOHN E. ALEXANDER, AND GOSTA GENBERG, OF PORT EDWARDS, WISCONSIN, ASSIGNORS TO NEKOOSA-EDWARDS PAPER COMPANY, OF PORT EDWARDS, WISCONSIN, A CORPORATION OF WISCONSIN.

## PROCESS FOR MAKING PAPER PULP.

No Drawing.

Application filed September 2, 1922. Serial No. 586,037.

*To all whom it may concern:*

Be it known that we, BERTRAM T. MCBAIN and JOHN E. ALEXANDER, citizens of the United States, and GOSTA GENBERG, a subject of the King of Sweden (who has declared his intention of becoming a citizen of the United States), all of whom are residents of Port Edwards, in the county of Wood and State of Wisconsin, have invented certain new and useful Improvements in a Process for Making Paper Pulp; and we do hereby declare that the following is a full, clear, and exact description of the same.

This invention relates to the production of wood pulp such as is used for making white paper from wood. The invention relates more particularly to the treatment of coniferous wood or other woods that are rich in rosin or similar substances which ordinarily produce dark colored pulp. Because of the continually increasing scarcity of such woods as spruce that lend themselves to the manufacture of bleached sulphite pulp, it is desirable to find a way to make white paper from woods like southern pine that must be treated by the sulphate process. Woods of this kind, however, yield a dark colored pulp which even after excessive bleaching remains of an undesirable color. Moreover, such excessive bleaching makes a very weak paper. The pulp made by the sulphite process is easily bleached but makes paper of less strength.

It is an object of the present invention to secure the easy bleaching quality of sulphite pulp and the strength of paper from sulphite pulp.

It is a further object of this invention to provide a method by which wood that requires the sulphate treatment may be made to produce paper which will be nearly white without the use of enough bleaching to materially impair the strength of the paper.

It is a further object of this invention to produce white paper from kraft pulp.

It is a further object of this invention to make use of the bleaching action of sulphite acid for the treatment of pulp which has been prepared by a sulphate process.

It is a further object of this invention to produce a method whereby paper, having the strength of brown kraft paper and the color of paper made by the sulphite process

from deciduous wood, may be produced from coniferous wood. 55

It is a further object of this invention to produce a paper by the sulphite process without the necessity of carefully separating all knots, bark or partially decayed wood as has heretofore been necessary when preparing white paper by said process. 60

Other and further important objects of the invention will be apparent from the disclosure in the following description, which sets forth the preferred form of our invention. 65

In making pulp according to our invention, the wood is first cut to appropriate sized chips by machines such as are already familiar to workers in this art. It is not necessary, however, to separate the bark, knots, partly decayed wood or other sources of dark color with the care which would be needed if the ordinary sulphite process were used. It is sufficient to make such separation as is usually required for the production of dark brown or kraft pulp by the sulphite process. 75

The chips thus prepared are cooked according to the usual sulphate process, the sulphate liquor being made up by the use of water and white liquor principally, as little black liquor as possible being employed. The sulphate pulp may be transferred directly from the sulphate cooker to a sulphite cooker, and washed therein, or the sulphate pulp may be first subjected to washing and lapping and the sheets may then be shredded and the shredded pulp introduced into the sulphite cooker. If desired, instead of sulphate pulp prepared in the way just described, ordinary commercial sulphate pulp may be employed. 80 85 90

When the sulphate pulp has been put in the sulphite digester, sulphite acid is used. 95 Preferably this acid should have approximately 4% for its total  $SO_2$  content of which about one quarter is in combined form as sulphite of calcium, and sufficient acid should be added to the pulp to make the contents of the digester have about the density corresponding to 10% of pulp. A higher density is to be avoided, because good circulation cannot be secured with it. The contents of the digester are cooked for about 100 three and a half hours. The temperature 105

should be gradually raised to a maximum of 300° F. The pressure should rise rapidly to about 70 pounds, this point being reached as soon as possible, instead of a lower pressure being maintained during the first two-thirds of the cooking time as is the practice in treating chips. The pressure should not at any time rise much above 80 pounds. If necessary, in order to keep the pressure below this figure, escape valves leading into the usual gas recovery main should be provided at the top of the digester, but no side release valves should be used.

When the cooking is completed the pulp is blown into the usual receiving tanks and there drained and washed in the usual manner. The recovered liquor may be used over again by being mixed with the sulphite acid. After the pulp has been sufficiently washed, it is made into sheets by being passed over lapping machines in the usual way.

Bleaching powder or other bleaching agent may be added either in the blow tank or during the lapping or at a later stage as desired. While the pulp is being bleached, care should be taken to avoid too high a temperature. The bleaching temperature ought not at any time to exceed 95° F. This is to make sure that no waste of chlorine, through the formation of chlorate, occurs.

The pulp made by this process may be used upon a paper machine and produces a sheet of paper sufficiently light colored for use as news printing or even as writing paper. The sulphite acid acts not only to directly lighten the color of the paper by its action upon the lignine and other darkening substances but also by so changing some of these substances that they are more easily bleached by the chlorine or other bleaching agent used in the after treatment.

It is to be understood that although we have described the treatment of the sulphate pulp by cooking in a sulphite digester, the bleaching results obtained by the use of sulphite acid may be obtained by mixing sulphite acid with the pulp in the blow tank or by sprinkling sulphite acid on the pulp on the wet machine, or by applying sulphite acid to the pulp in any other desired way. It is further to be understood that numerous

details of the process may be varied through a wide range without departing from the spirit of this invention, and we do not desire limiting the patent granted otherwise than is necessitated by the prior art.

We claim as our invention:

1. The process of making a light colored paper from resinous wood, which comprises treating the wood by the usual sulphate process and then treating the resulting pulp with sulphite acid.

2. The process of making paper pulp which comprises treating resinous wood with an alkali sulphate solution and then treating the resulting pulp with an acid solution containing  $\text{SO}_2$ .

3. The process of making a strong white paper from kraft pulp, which comprises treating the pulp with a liquor of acid calcium and magnesium sulphite, and acting upon the result with a bleaching agent.

4. The process of making white pulp from sulphate pulp which comprises cooking the sulphate pulp in a digester with sulphite acid at a pressure between 50 and 80 pounds and at a temperature above the boiling point of water for a period exceeding two hours.

5. The process of making white pulp from sulphate pulp which comprises cooking the sulphate pulp in a digester with sulphite acid at a pressure between 50 and 80 pounds and at a temperature above the boiling point of water for a period exceeding two hours, separating the resulting pulp from the sulphite liquor, and washing and bleaching the pulp.

6. The process of making a light colored paper from dark sulphate pulp which consists in treating the sulphate pulp in a digester with sulphite acid.

7. The process of making a light colored paper from dark sulphate pulp which consists in treating the sulphate pulp in a tank with sulphite acid.

In testimony whereof we have hereunto subscribed our names.

BERTRAM T. MCBAIN.  
JOHN E. ALEXANDER.  
GOSTA GENBERG.